

Aug. 19, 1924.

1,505,127

H. D. AYRES

WOVEN FABRIC TEST PIECE AND METHOD OF TESTING WOVEN FABRIC

Filed Feb. 9, 1920



Inventor  
H.D. Ayres  
By Robert M. Pearson  
Atty.

Patented Aug. 19, 1924.

1,505,127

# UNITED STATES PATENT OFFICE.

HIRAM D. AYRES, OF AKRON, OHIO, ASSIGNOR TO THE B. F. GOODRICH COMPANY, OF NEW YORK, N. Y., A CORPORATION OF NEW YORK.

## WOVEN-FABRIC TEST PIECE AND METHOD OF TESTING WOVEN FABRIC.

Application filed February 9, 1920. Serial No. 357,315.

*To all whom it may concern:*

Be it known that I, HIRAM D. AYRES, a citizen of the United States, residing at Akron, in the county of Summit and State 5 of Ohio, have invented a certain new and useful Woven-Fabric Test Piece and Methods of Testing Woven Fabric, of which the following is a specification.

This invention relates to the art of testing 10 woven fabric such as that used for making pneumatic tires or that used for making balloon envelopes, which fabric as it comes from the loom is often or usually in an unbalanced condition as respects the amount 15 of crimp in the warp and filler, respectively, and hence lacks a maximum degree of suitability for its intended purpose. The object of my invention is to provide an improved form of fabric test-piece, an improved 20 method of preparing and an improved method of using the same, for the purpose of determining the characteristics of the fabric in one or more of its various stages,—for example, in its uncoated condition as it 25 comes from the loom, in its rubberized condition before application to purposes such as tire making, and in its condition after use in the tire or other article. This determination affords information to the manufacturer of articles made from the fabric, 30 such as tires, which permits the intelligent application of expedients, either during or after the weaving of the fabric, tending to correct the usual inequalities. The principal 35 inequality commonly found in tire fabric, for instance, consists in a greater degree of crimp in the warp threads than exists in the weft or filler threads, owing to the methods used in weaving, so that 40 when the two sets of threads are subjected to equal elongations in an inflated tire, the warp threads, being more stretchable than the filler threads, are subjected to a less degree of strain.

45 The accompanying drawing shows in elevation, partly broken away, a test-piece of fabric prepared and mounted according to my invention, together with the grips through which the desired loading is applied to the two sets of threads.

50 This test-piece is made in the shape of a Greek cross, with four arms 10, 10 of approximately equal length, and a central quadrilateral 11, which for convenience may 55 be termed a "square," although the two sets

of threads in the fabric when taken from a pneumatic tire, for example, are often at an angle to each other other than a right-angle. The cross-shaped test-piece is detached from a sheet of woven fabric by cutting the arms, 60 at their sides, parallel to the longitudinal threads of said arms, and at their ends, across said longitudinal threads, and some of the intermediate cross threads are then drawn for a purpose to be described. In 65 testing this fabric piece I prefer to hang it in a vertical plane with the band of warp threads 12 running vertically and the band of filler threads 13 horizontally, or at a slight angle to the horizontal if the piece to 70 be tested is taken from a portion of a structure such as a tire, where the two sets of threads lie at other than a right-angle to each other.

75 14, 14 are grips or clamps, four in number, applied to the ends of the arms of the fabric test-piece, and each comprising a pair of stout plates or flat bars 15, held against the fabric by bolts 16 and roughened on their inner surfaces as indicated at 17 in order to increase their hold upon the fabric. To the members of each pair of grips 14 oppositely-pulling forces are applied by means of draw-bars 18, whose inner ends are 80 represented in the drawing lying between the plates of the grips and engaging their middle portions by means of pins 19, this middle point of application of the pulling forces being especially desirable when testing non-rectangular fabric taken from a 85 tire. The elongation of the warp or filler threads, or both, due to the loading forces, is observed by making suitable marks on the fabric and noting their increment of length or amount of shifting of position as the 90 loads are increased. The loading forces may be of any suitable character such as weighted cords or chains passing over pulleys, and the application of the weights and observation of measurements on the fabric test-piece may be performed in any suitable way.

100 The portions of the fabric test-piece engaged by the grips 14 contain both sets of threads in order to retain the proper form of such portions and increase the adhesion of the grips upon the longitudinal threads which are being subjected to strain. Between the grips and the central test-square 11 the cross threads in each arm 10 are removed or drawn. Heretofore, in the testing 105 110

of fabric by means of cross-shaped test pieces to whose arms various loads are applied, the cross threads have been left in the arms between the grips and the central 5 square and the effect has been to contract the width of said arms owing to the increasing crimp of the cross-threads when tension is applied to the longitudinal threads, with the consequence that uncertain 10 readings of elongation are obtained in the central test-square, the corners of this square are over-strained and the fabric threads break at these corners before the limit of strength of the middle is reached. 15 When the cross threads are drawn in accordance with my invention these troubles are obviated.

The fabric test-piece when strained to the limit of strength of its threads should theoretically break in the woven central square 20 rather than in the unwoven threads of the arms 10, for the reason that the straight threads in these arms are subjected to a force only equal to the longitudinal force acting 25 in the plane of the fabric, whereas the crimped threads in the central square are subjected to resultant forces acting at an angle to the plane of the fabric along the sides of the waves or undulations forming 30 the crimps, which forces are greater than the force acting in the plane of the fabric. Experience confirms theory, as it is found that the threads will break in the majority 35 of cases in the woven fabric of the central square.

It will be obvious from the description thus far given that I have devised a form of fabric test-piece and a mode of using the same by which the manufacturer of articles such as tires made from the fabric is 40 enabled to obtain useful information as to the characteristics of such fabric which will, if desired, enable corrections to be made improving its quality either in the weaving of 45 the same or in the treatment of the fabric after it is woven. For example, if by applying equal loads to the warp and filler threads of the test-piece it is found that the warp threads stretch a certain percentage 50 more than the filler threads, or if by imposing equal amounts of elongation upon the warp and filler threads it is found that a certain less increment of weight is required to impose this elongation upon the 55 warp threads than is required for the filler threads, the user of my invention will know that a correspondingly greater amount of crimp exists in the filler than in the warp. It is found in practice that the amount of 60 unbalance of the fabric in this respect varies greatly according to the particular mill from which the product comes, and as it is usually to the tire-manufacturer's advantage to buy his fabric from various sources, it is desirable for him to be able to treat the fabric 65

from these different sources in such manner as to bring it all to a condition of uniform or known degree of balance. This can conveniently be done in connection with the operation of applying the coating of rubber 70 to the fabric in a calender, and I prefer to perform it by means of the automatic fabric-tensioning device forming the subject-matter of an application, Serial No. 357,814, filed concurrently herewith. It may, on the other hand, be possible to obtain a balance of extensibility between the warp and the 75 filler in the course of building the pneumatic tire casing, although this would be somewhat difficult. Even if nothing is done toward obtaining such balance, this invention may afford the tire manufacturer information useful to him in connection with the acceptance or rejection of fabric or in the combining of fabric from different portions 80 of the same roll which vary in their characteristics, in making up tire carcasses composed of several plies or laminations.

In the operation of my invention, the application of loads upon the fabric test-piece 85 and the taking of readings of elongation in the central test-square may be done according to various plans of procedure, which can largely be left to the judgment and skill of the operator. The mode which I prefer, but which can be varied as circumstances or choice may demand, is to first lay out the fabric test-piece flat upon a smooth surface and mark horizontal and vertical lines of predetermined length near 90 the two edges thereof. Adjacent to these lines two steel rules graduated in small dimensions are attached to the fabric, one end of each rule having a fixed attachment and the other being supported in such manner 95 that the fabric may slide with respect to the rule so that the amount of increase in length of the marked lines along the warp or the filler can be observed against the graduations on the rule, the readings being preferably taken by two observers through microscopes on opposite sides of the test-piece 100 when the latter is suspended in a vertical plane. In placing the fabric in the grips, the portions of the arms 10 engaged by the 105 grips are somewhat stretched laterally as indicated in full lines in the drawing, so that when the warp and filler are stretched nearly to the breaking point, giving the test-piece approximately the outline shown by the dotted lines 20 in the drawing, there will not be too great a departure from parallelism in the threads of said arms as between those threads in the middle and those 110 at the sides of the arms. In using the method of equal elongations, the effort is made to apply the loads very nearly simultaneously upon the warp and filler threads 115 in such respective degrees as will maintain their elongations the same. For example, 120

- after applying a small minimum load, such as five pounds, to the warp 12, balancing this with a co-ordinate load on the filler, and observing and recording the elongations corresponding to this first load on each set of threads, I then prefer to load the filler by successive predetermined amounts, such as 25, 50, 100, 200, etc., pounds, bringing the warp as nearly as possible simultaneously to an elongation equal to that caused by the filler load, noting this elongation and also the amount of the filler load and then proceed to the next loading, and so on until the fabric test-piece breaks.
- 15 The recorded observations may afterwards be plotted in the form of a curve or curves, if it is desired to display the results graphically, and a study of these results enables the tire-maker to apply the necessary corrections to the fabric or otherwise usefully to employ the information obtained, as already pointed out.
- 20 The details of procedure may, of course, be considerably varied without departing 25 from my invention.

I claim:

1. A woven-fabric test-piece in the form of a cross with free ends, having the transverse threads withdrawn from its arms adjacent to the central quadrilateral.
  2. A woven-fabric test-piece in the form of a cross with free ends, the arms of said cross adjacent to the central quadrilateral having their transverse threads withdrawn, 35 and said arms adjacent to their ends having the transverse threads in place.
  3. A woven-fabric test-piece in the form of a cross having a substantially equal number of warp and filler threads, said cross 40 having arms with free ends, the portions of said arms adjacent to the central square being free from transverse threads.
  4. The method of preparing a woven-fabric test-piece which comprises detaching 45 from a sheet of fabric a piece in the form of a Greek cross, with the warp and filler threads parallel to the arms of the cross and substantially equal in number in both sets, and withdrawing the transverse
- threads from the arms adjacent to the central square.
5. The method of testing woven fabric for characteristics of warp and filler which comprises preparing a cross-shaped test-piece with warp and filler threads running longitudinally of the respective arms and having the transverse threads withdrawn from said arms adjacent to the central quadrilateral, loading one of said sets of threads in a definite manner and observing the resulting elongation.
6. The method of testing woven fabric for characteristics of warp and filler which comprises preparing a cross-shaped test-piece having warp and filler threads running longitudinally of the respective arms, applying a known load to one set of threads, applying such a load to the threads of the other set as to elongate the latter by substantially the same amount as the first set, and observing the amount of the last-said load.
7. The method of testing woven fabric for characteristics of warp and filler which comprises preparing a cross-shaped test-piece having a substantially equal number of warp and filler threads running longitudinally of the respective arms, withdrawing the transverse threads from the four arms in zones between the outer end portions of said arms and the central square, applying grips to said outer end portions, applying a series of known weights through one pair of grips to the threads of one set and observing the resulting elongations of a measured portion of one of said threads in the central square, applying such weights through the other pair of grips to the threads of the other set as will cause successive elongations of an equal measured portion of one of the threads of the other set in said square substantially equal to the respective elongations of the first set, and observing the amounts of the several weights thus applied to said second set.

In testimony whereof I have hereunto set my hand this 5th day of February, 1920.

HIRAM D. AYRES.